

March 17, 1959

J. S. TURNBULL

2,877,523

VACUUM CASTING

Filed Aug. 29, 1955



FIG.1



FIG.2

INVENTOR

John Stretton Turnbull

By *Rossie & D'Amico*

ATTORNEYS

# United States Patent Office

2,877,523

Patented Mar. 17, 1959

1

2,877,523

## VACUUM CASTING

John Stratton Turnbull, Bowdon, England, assignor to Metropolitan-Vickers Electrical Company Limited, a British company

Application August 29, 1955, Serial No. 531,028

Claims priority, application Great Britain September 3, 1954

2 Claims. (Cl. 22—73)

This invention relates to vacuum casting, that is to say, to methods of casting wherein the mould is subjected to suction or evacuation to a desired degree during the pouring of the metal or other material to be cast.

In the casting art, it is in general necessary that the gas or air be removed from the mould cavity at a higher rate than that at which the molten metal enters the cavity, in order that the latter may be filled without it being necessary to provide risers or make other provisions which in general are objectionable or disadvantageous. It has therefore been necessary to make careful arrangements in regard to pouring the molten metal without turbulence, bottom-gating and choke-feeding, for example, since the permeability of the mould is usually so low that the gas or air cannot be expelled from the mould cavity except by special channels or passages. With the above considerations in mind, it has been proposed to subject the mould to suction or vacuum but the use of such vacuum casting has been limited because in general it is only possible to apply the suction to one or two faces of the usual rectangular mould and the evacuating equipment is required to withdraw the air or gas from the mould cavity through a considerable thickness of the material forming the mould.

The present invention has for its object to provide a method of vacuum casting wherein the disadvantages set forth above may be obviated. The invention is eminently, but not exclusively, applicable to the so-called "precision casting."

The method of vacuum casting according to the present invention comprises supporting a permeable shell mould within a container by means of permeable supporting means between the outer surface of the shell and the inner surface of the container, connecting the container with a vacuum accumulator and evacuating pump with valve means between the container and the accumulator, evacuating the accumulator with the valve means closed, and subsequent to said evacuation of the accumulator, opening said valve means and pouring the metal or other casting material into the mould as a combined operation, that is to say, more or less simultaneously.

The supporting means referred to preferably comprises packed granular material of angular form and of large size, such as hereinafter indicated. The composite material formed by the shell and the supporting means is designed for maximum or high flow of air or gas from the mould cavity or cavities within the shell directly from the inner surface of each cavity through the permeable wall of the shell. Since a permeable shell mould is employed, that is to say, a mould which has an outer shape conforming substantially to the general shape of the mould cavity, or cavities in the case of a complex casting, the arrangement is therefore such that the air or gas can pass freely through the shell wall on all or substantially all surfaces of the mould cavity or cavities. Since the accumulator is evacuated prior to the casting operation and with the valve means closed, a comparative small evacuating pump is enabled rapidly to evacuate

the mould cavity or cavities of air or gas, it being understood that the accumulator has a capacity many times that of the mould cavity or cavities.

Preferably the pump is left running during the casting operation and solidification of the casting, whereby to balance leakage of air into the container when the mould is full of the poured metal. By this means also decarburisation of the surface metal of the casting and formation of oxides therein, which normally result from the contact of the poured metal with the atmospheric gases in the mould, are avoided, since the atmospheric gases are withdrawn from all or substantially all the surfaces of the mould cavities. Further with a view to reducing such leakage, the shell is preferably provided with a pouring throat which is sealed externally thereof with respect to an opening in the container, the throat extending through said opening.

The shell may be formed by various methods, but is preferably in accordance with the invention set forth and claimed in copending United States application Ser. No. 319,776, filed November 10, 1952, now U. S. Patent No. 2,815,552, issued December 10, 1957 to John Stratton Turnbull and Richard Glyn Nicholas, assignors to Metropolitan-Vickers Electrical Company Limited.

The invention also includes within the scope thereof apparatus for carrying out the method hereinbefore set forth, said apparatus comprising a permeable shell mould arranged within a container and supported therein by permeable supporting means between the outer surface of the shell and the inner surface of the container, a vacuum accumulator and an evacuating pump for evacuating said accumulator, and a connection between said accumulator and said container, said connection including valve means for controlling the passage of air or gas from the container into the accumulator.

Reference will now be made by way of example to the accompanying drawing, in which:

Fig. 1 is a cross-sectional elevation showing diagrammatically one arrangement of mould for carrying out the method of casting according to the invention, and

Fig. 2 is a diagram illustrating the mould of Fig. 1 arranged in apparatus according to the invention.

In Fig. 1, a shell mould 1 of the desired object to be cast is made such as by the method according to the aforementioned U. S. application No. 319,776/52, now U. S. Patent No. 2,815,552, issued December 10, 1957. This mould is positioned in a metal container 2 and invested therein with a coarse dry refractory aggregate of angular nature indicated by the cross hatching 3. The aggregate may for example have a particle size of between one-quarter and one-half of an inch.

The mould is provided with a pouring throat 4 which extends through the open top of the container. The top of the mould, with the exception of the pouring throat 4, has built up thereon a collar 5 of solid investment extending from the external surface of the throat to the sides of the container 2, thereby completing the enclosure of the mould 1 and the refractory aggregate 3. The collar may be formed from a thick viscous ceramic slurry poured or moulded round the throat 4 of the mould onto the top of the refractory investment 3, the slurry being so turgid as not to flow into the interstices between the particles of the investment. The slurry is preferably alcohol based so as to stiffen rapidly. The collar 5 is made of substantial depth, for example one inch or more, whereby to minimise leakage of air into the container by way of the permeability of the collar when the container is evacuated.

Means are provided for evacuation of the container, and, in the arrangement illustrated, these means comprise a pipe 6 having a bore, for example of one inch,

welded into one side of the container and connected such as by a rubber tube or hose to the evacuating pump or accumulator.

In Fig. 2, the rubber hose is indicated at 7 and connects the pipe 6 with a pipe 8 in turn connected with a vacuum accumulator 9, a valve 10 being included in the pipe 8. The accumulator 9 is connected directly with an evacuating pump 11. Alternatively, the container 1 may be provided with a bottom wall having a number of orifices therein and the mould may be placed on a vacuum stillage incorporating a pump accumulator, and valve means, so that in operation the air or gas may be drawn through said orifices.

The vacuum accumulator 9 with which the pipe 6 or the vacuum stillage is connected may have for example a volume of twenty to thirty times that of the mould cavity.

When casting, the mould may be either hot or cold according to conditions and requirements. When the mould is employed hot, then with the second method of evacuation just above indicated, the metal tube protruding from the container is chilled-off before being connected with the rubber tube or hose.

In making the casting, the accumulator is first evacuated to the desired degree without drawing air from the mould, valve means between the accumulator and the container being closed at this time. At, or approximately at, the instant when pouring of the metal into the mould is commenced, said valve means are opened and the vacuum previously built up in the accumulator is then applied to the container so as to obtain a high rate of extraction of air and gas from the mould cavity as the molten metal begins to flow down the throat. It will be understood that the use of the accumulator and opening of the valve means only at the time at which the casting is commenced enables a relatively small and economical evacuating pump to be employed. The use of a shell mould and highly permeable backing enables the air or gas to be extracted rapidly by the vacuum from the mould cavity or cavities.

The valve means is left open for the necessary time required for the cast metal to solidify, which time may for example be of the order of five minutes. The pump is left running during this time so as to balance any leakage of air through the wall of the pouring throat and the collar by which the throat is sealed to the walls of the container at the upper end thereof.

The process according to the invention, whilst having general application, is eminently applicable for the precision casting of long and thin objects of simple or complex shape, and enables a high surface finish or definition to be obtained.

As well understood in the art, long castings of relatively small sectional thickness or area are difficult to fill completely with poured metal without trapping gas, obtaining miss-run edges and other defects. The invention also enables alloys which might otherwise be regarded as uncastable to be cast with considerably improved results. In casting alloys, which in general provide inferior surface finish by the normal casting processes as a result of high viscosity of the molten metal and consequent tendency to the trapping of small gas pockets on the surface of the casting, the invention overcomes these defects and in general enables castings

having good definition to be obtained where not possible by the usual methods.

What I claim as new and desire to secure by Letters Patent of the United States is:

- 5 1. An apparatus for use in the precision vacuum casting of relatively long thin objects comprising a substantially air-tight container confining a body of readily gas permeable material, a one-piece elongated readily gas permeable shell mold mounted in said container and conformably embedded in said body of material, said mold forming at least one relatively narrow cavity and having a pouring throat projecting above said container through an opening provided therein and including a relatively narrow throat section communicating with said cavity whereby poured casting material in molten state fills said throat to seal the cavity substantially air-tight in said container, an exhaust conduit extending through the container into said body of material, an accumulator having a volumetric capacity at least many times that of said mold and said container, a vacuum pump connected to said accumulator, and a valve in the conduit between said container and the accumulator said valve being normally closed in said apparatus to permit said accumulator to be evacuated and conditioned for sudden and continuing application of its vacuum to the interior of said container when said valve is opened.
- 10 2. In a vacuum casting process for use in producing relatively long thin objects the steps of providing an upright relatively narrow one-piece gas permeable shell mold embedded in a confined relatively coarse conformable gas permeable support medium in a substantially air-tight container and having a relatively narrow pouring throat section projecting beyond the container, accumulating vacuum in a source having a volumetric capacity many times that of the cavity in the mold and container, sealing the cavity within the container by pouring molten casting material into the mold to fill up the relatively narrow throat section while substantially at the same time rapidly and substantially evacuating said
- 15 30 mold through substantially all faces of said cavity by suddenly applying the accumulated vacuum of said source to said confined support medium, and continuing to apply a vacuum to evacuate the interior of said container as molten casting material fills said mold to substantially evacuate leakage of air into said container.
- 20 35 40 45

#### References Cited in the file of this patent

#### UNITED STATES PATENTS

|    |           |             |                |
|----|-----------|-------------|----------------|
| 50 | 1,708,011 | Crowley     | Apr. 9, 1929   |
|    | 2,117,114 | Hazey       | May 10, 1938   |
|    | 2,379,401 | Poulter     | June 26, 1945  |
|    | 2,434,780 | Wiss et al. | Jan. 20, 1948  |
|    | 2,660,770 | Davis       | Dec. 1, 1953   |
|    | 2,718,041 | Georgen     | Sept. 20, 1955 |

#### FOREIGN PATENTS

|           |               |                |
|-----------|---------------|----------------|
| 716,251   | Great Britain | Sept. 29, 1954 |
| 1,039,893 | France        | May 20, 1953   |

#### OTHER REFERENCES

Fiat Final Report No. 1168 entitled "The 'C' Process of Making Molds and Cores for Foundry Use," by W. W. McCullough, published by the Office of Technical Services, Dept. of Commerce, Washington, D. C.